# EUROPEAN PATENT SPECIFICATION

(11) **EP 0 581 962 B1**
(45) Date of publication and mention of the grant of the patent: **09.04.1997**
(21) Application number: 93902521.9
(22) Date of filing: 22.01.1993
(51) Int. Cl.: B05C 5/02, B05C 5/00, B05D 1/26, B05D 1/30, G03C 1/74

(54) **METHOD OF AND DEVICE FOR APPLICATION**
AUFTRAGSVERFAHREN UND -VORRICHTUNG
PROCEDE ET APPAREIL D'APPLICATION

(30) Priority: 22.01.1992 JP 9357/92; 20.08.1992 JP 221564/92
(43) Date of publication of application: 09.02.1994
(73) Proprietor: KONICA CORPORATION, Tokyo 163 (JP)
(72) Inventor: YOSHIDA, Makoto, Hino-shi, Tokyo 191 (JP); SAKATA, Kazuhiko, Hino-shi, Tokyo 191 (JP); SHIMIZU, Kazuyuki, Hino-shi, Tokyo 191 (JP); TANAKA, Takeshi, Hino-shi, Tokyo 191 (JP)
(74) Representative: Henkel, Feiler, Hänzel & Partner
(86) International application number: JP9300081
(87) International publication number: WO9314878

(56) References cited:
- JP-A- 3 138 376
- JP-A-59 047 399
- JP-A-59 189 963
- Microfilm of the specification and drawings annexed to the written application of Japanese Utility Model Application No. 48251/1989 (Laid-Open No. 142667/ 1990), (Mitsubishi Heavy Industries, Ltd.), December 4, 1990 (04.12.90), p. 6, l. 3 - l. 10 (Family: none)

## Description

### FIELD OF THE INVENTION

The present invention relates to a coating apparatus of a hopper type and to a coating method as defined in the preamble of claim 1 and 7, respectively.

### BACKGROUND OF THE INVENTION

Coating apparatus of a slide hopper type and those of an extrusion hopper type are capable of performing high-speed coating, thin-layer coating and simultaneous multilayer coating, and some of them are used widely for photographic light-sensitive materials and others are used for magnetic recording materials widely, depending on their features. On coating apparatus of this type, a staying coating solution which is called a bead of a coating solution is formed between a coater tip (also called an edge or a lip) and a running flexible support (also called a web), and coating is performed through the bead.

On such a bead coater, stability of coating is extremely influenced by stability of the bead. The stability of the bead is influenced by factors including the distance setting up between a lip and a web, environmental conditions and physical properties of a coating solution, namely viscosity and surface tension. In the case of simultaneous multilayer coating, in particular, the relation of physical properties between layers greatly affects the bead stability, and when the coating speed is high, or when a coated layer is thin, it is difficult to secure the bead stability. In the case of an unstable bead, coating defects are caused such as pencil lines, streak defects and coating solution shortage.

For an improvement of such bead stability, there is known, for example, a method to provide a pressure difference between the upper portion and the lower portion of a bead. To be concrete, there has been taken a measure wherein a decompressed chamber is positioned below a bead to attract the bead downward, and thereby to improve the bead stability.

However, in the case of a coating solution having extremely low viscosity, for example, a coating solution having a viscosity of 10 cps or less, containing an organic solvent and having low surface tension, there have been some occasions wherein the coating solution oozes out of a lip portion other than the bead, and drips on a coated layer or on a support despite the above-mentioned measure, causing comet defects and dropping defects, or causing more streak defects even when the coating speed is not so high and a coated layer is not so thin.

For the problems mentioned above, it is suggested in Japanese Patent Publication No. 57629/1989 that a lip portion on the tip of a coating apparatus is provided with water-repellent resins. However, even when fluorine-containing resins are provided on the lip portion and the surface thereof is ground, for example, it is difficult to obtain satisfactory accuracy and strength on the lip portion due to the strength of the resins because the lip portion is required to have an extremely high accuracy. Therefore, it is difficult to obtain accuracy for a uniform coating layer thickness and scratches are easily caused, thus, it is difficult to maintain stable coating conditions.

From JP-A 59 189 963 there is known a coating applicator of a hopper type for coating a coating liquid on a running support in which a water-repellent fluororesin polyacetal resin is applied onto the top end of the applicator head at the lower end of a slide surface to thereby inhibit the falling-in of the coating liquid at the lower end of the slide surface by the effect of water repellancy.

An ink jet recording head is described in JP-A 3 274 163 in which a nozzle plate is formed by an electroless plating casting method and a fluoro high polymer eutectoid plating of tetrafluoroethylene fine particles is performed on said surface to improve the removal of residue of ink therefrom.

### OBJECT OF THE INVENTION

To overcome the problems mentioned above, the object of the invention is to provide a coating apparatus of a hopper type and a coating method which cause no coating defects including streak defects and are hardly scratched even in the case of coating with a coating solution having low surface tension and viscosity.

### DISCLOSURE OF THE INVENTION

The object of the invention mentioned above can be achieved by a coating apparatus of a hopper type for coating one or more kinds of coating solutions on a running flexible support, said coating apparatus being provided with a slit and a lip portion at the tip of a hopper,
characterized in that only an inclined surface following the lip portion is subjected to composite plating to be covered by a coat of the plating in which fluorine-containing resins are dispersed in a form of eutectoid such that the length of a bead upstream the slit in the running direction of the flexible support is adjusted to be nearly the same as that of the lip portion at the tip of the hopper at the upstream side of the slit in the running direction of the support.

According to the invention there is also provided a coating method comprising a step for coating one or more kinds of coating solutions on a running flexible support, wherein a coating apparatus is used which is provided with a slit and a lip portion at the tip of a hopper and in which an inclined surface portion following the lip portion at the tip of a hopper is provided with a coat of composite plating wherein fluorine-containing resins are dispersed in a form of eutectoid,
characterized in that the coating is performed under the condition that a length of a portion of a bead upstream the slit in the running direction of the flexible support is adjusted to be nearly the same as the length of the lip portion at the tip of the hopper at the upstream side of the slit in the running direction of the flexible support in that only the inclined surface following said lip portion is subjected to the composite plating.

Preferred embodiments of the apparatus and the method are defined in the subclaims.

Incidentally, it is preferable that the aforementioned coat of plating wherein fluorine-containing resins are made in a form of eutectoid is one plated with nickel through non-electrolytic plating utilizing a chemical reaction, and it is preferable that the coat of plating is subjected to heat treatment at a temperature of not less than 300°C.

### BRIEF DESCRIPTION OF THE DRAWINGS

Fig. 1(a) Explanatory sectional view showing oozed out solution on an extrusion coating die
Fig. 1(b) Explanatory plan view show oozed out solution on a coater of an extrusion hopper type
Fig. 2(a) Sectional view of a coater of a slide hopper type
Fig. 2(b) Sectional view of a coater of an extrusion hopper type
Fig. 2(c) Sectional view of a curtain coater (of a slide hopper type)
Fig. 2(d) Sectional view of a curtain coater (of an extrusion type)
Fig. 2(e) and Fig. 2(f) illustrations showing the relation between a length of a lower portion of a bead and that of a lip at an upstream side.

A detailed description of the invention will be given as follows.

The inventors of the present invention recognized the difficulty of coating stably when coating a coating solution having low surface tension and low viscosity, for example, a coating solution of an organic solvent type by the use of a bead-employing coating apparatus such as a coater of a slide hopper type or an extrusion coater. The inventors presumed that the cause of the difficulty lies in the under mentioned mechanism.

A coating apparatus such as a coater of a slide hopper type, a coater of an extrusion hopper type or a curtain coater is usually made of metal, especially of stainless steel. It has been made clear that wettability of a coating solution having low surface tension and low viscosity such as an organic solvent for metal is very high because the surface energy of metal is large and its critical surface tension is high. Therefore, a coating solution spreads over the surface of the metal and thereby a bead can neither be formed sufficiently nor be kept in a stable form, and thus, the coating solution spreads over the lip or its surroundings.

When a coating solution spreads more briskly, the coating solution oozes out even on an inclined surface following the lip portion where the coating solution gathers and drips on the coated layer or on the support, causing dropping defects problems.

Fig. 1 (a) is an illustrative sectional view showing an example of oozing out, and Fig. 1 (b) is a plan view. In the figure, the numeral 1 represents an extrusion coating die and 10 represents a slit through which a coating solution is supplied. The numeral 11 is a front bar and 12 is a back bar. Between web 2 running in the arrowed direction and the front and back bars, there is formed bead 13 through which a coated layer is formed on a web. In this case, oozing out of the coating solution impedes complete bead formation, and oozed out portion 14 is formed under the regular bead. When the oozed out portion grows larger, it touches the web, causing streak defects or comet defects, or causing edge dirt at uncoated portions on both sides of the support, or the oozed out portion causes a dropping defect.

The problems mentioned above are caused not only in a bead coater but also in a curtain coater. In a curtain coater, no bead is formed but a coating solution flows downward in the form of a curtain to hit a web, and the force of hitting the web causes a coated layer to be formed on the web. Even in this case of a curtain coater, there are two types, one is an extrusion type and the other is a slide hopper type. In the case of the former type, the coating solution oozes out on a lip as well as on an inclined surface following the lip at the slit outlet from which a flow-down layer comes out, and the oozed coating solution disturbs liquid releasing at the slit outlet, causing streak defects on the flow-down layer, or the oozed coating solution forms a drop which gets on the flow-down layer or drops on the web, resulting in dropping defects and streak defects.

Even in the case of a curtain coater of the slide hopper type, a coating solution oozes out on a beak-shaped lip portion and on its reverse side, and there are similar problems to those occurring on an extrusion coater.

To avoid such phenomenon of oozing out of a coating solution, it is necessary to use, as a lip portion and/or an inclined surface following the lip portion in a coating apparatus, a material having small surface energy and low critical surface tension whose water-repellent action prevents wetting, spreading and oozing out of a coating solution.

Though water-repellent resins such as Teflon or the like are used as an actual means for giving water-repellent property to a lip portion according to Japanese Patent Publication No. 57629/1989, it has been made clear that it is difficult to obtain the precision necessary for the lip of a hopper and to maintain the precision without damaging the lip even when a grinding step is taken for finishing the lip in the means for providing resins in the lip, although it is expected that Teflon is excellent in water-repellent property and it prevents a coating solution from oozing out and thereby prevents streak defects.

In the invention, it was found that composite plating wherein fine particles of fluorine-containing resin such as Teflon are dispersed in a form of eutectoid is very effective as a means which has water-repellent property and prevents streak defects and comet defects while correcting the aforementioned drawbacks. Due to the composite plating, it is possible to maintain the precision of a lip of a base material, which is a special feature of plating, and to form a coat having high hardness, while keeping the water-repellent property almost up to that of pure Teflon. A coating solution having low surface tension and low viscosity was coated at high speed by a hopper wherein a coat was formed on the surface of a lip portion and/or the surface of an inclined surface following the lip portion, and the occurrence of comet defects, streak defects and dropping defects were not observed at all.

Fluorine-containing resins to be made in a form of eutectoid are preferably those having excellent water-repellent property wherein a carbon chain in a polymer is covered by as many fluorine atoms as possible such as in polytetrafluoroethylene known as Teflon (made by Du Pont Corp. in the U.S.)

From the viewpoints of hardness, corrosion resistance and adhesiveness to a base material, it is preferable that nickel or chromium is used for a coat of plating wherein fluorine-containing resins is made in a form of eutectoid. It is further preferable that a lip portion for a coating die is plated by non-electrolytic plating utilizing a chemical reaction, from the viewpoints of uniformity of thickness of a plated coat, straightness and edge sharpness, which are required to be on a high level.

As a useful and concrete example of the so-called plating in the invention, there may be cited KANIFLON that is a trade name sold by Japan Kanigen Co., Ltd., as non-electrolytic nickel plating wherein Teflon fine particles, for example, are dispersed in a form of eutectoid. It is further possible to expect the effect of prevention of streak defects and others even for a coating solution having lower surface tension, due to more excellent water-repellent property obtained in the plating method developed by Applied Science Research Institute and C. Uyemura & Co., Ltd., wherein fluorine-containing resins are dispersed in a form of eutectoid.

After a coat of plating has been formed, it is preferable that the coat is subjected to heat treatment at a temperature of not less than 200°C, and it is more preferable that the coat is subjected to heat treatment at a temperature ranging from 300°C to 350°C. The purpose of the above is to decompose, through heat treatment, the dispersing agents used for dispersing fluorine-containing resins uniformly in a plating solution so that the dispersing agents staying on the surface even after the formation of the coat of plating may not impede the water-repellent effect.

Portions to be plated include a lip portion of a hopper and an inclined surface following the lip portion, and it is preferable for coating that a length of the lower portion of a bead is substantially the same as that of a part of the lip positioned at an upstream side.

Namely, it is preferable that a material having critical surface tension which is lower than surface tension of a coating solution is used on the surface of a lip situated at the tip of a hopper.

The coating solution, in this case, concretely includes those for a photographic light-sensitive material layer, especially a photographic foundation layer, a light-sensitive material for a lithographic printing plate, a magnetic recording material and its foundation layer or a backcoating layer, and an electrophotographic light-sensitive material and so on.

Fig. 2 (a) to (f) are illustrative diagrams showing various coating apparatus and locations where problems tend to happen, that is, locations shown with thick lines to which the plating of the invention is to be applied.

Fig. 2 (a) is a sectional view of a coater of a slide hopper type, Fig. 2 (b) is a sectional view of a coater of an extrusion hopper type, Fig. 2 (c) is a sectional view of a curtain coater of a slide hopper type, and Fig. 2 (d) is a sectional view of a curtain coater of an extrusion hopper type, and the coat of plating of the invention is applied to each location. For the reason mentioned above, it is preferable to employ a coating method wherein a bead is adjusted so that a length of the bead may be equal to that of a part of the lip situated at an upstream side when only the inclined surface following the lip portion is subjected to plating on a coating apparatus of a hopper type. Fig. 2 (e) represents an explanatory diagram showing a preferable length of a lower portion of a bead in the case that only an inclined surface portion following a lip is plated, for extrusion type coating, while Fig. 2 (f) represents that for slide hopper type coating.

### EXAMPLES

Effects of the invention will be illustrated as follows, referring to the examples.

### Example 1

A coat of nickel plating of about 10 µm thick wherein Teflon fine particles are dispersed in a form of eutectoid was applied to a lip portion of a slide hopper coating apparatus, and a coating solution having the following composition was coated on a polyethylene terephthalate web having a thickness of 100 µm and a width of 300 mm.

After coating under the conditions of coating speed of 50 m/min, decompression degree of -20 mmaq and coating density of 20 ml/m², neither coating defects such as streak defects or the like nor abnormal coating thickness were observed, resulting in stable coating.

| [Composition of coating solution] | parts by weight |
|---|---|
| Methyl ethyl ketone | 50 |
| Methanol | 30 |
| Ethyl acetate | 10 |
| Polymethylmethacrylate | 1 |

### Comparative example 1

After coating with a coater of the slide hopper type which is of the same type as in Example 1 but is not subjected to the aforementioned plating on its lip portion, there were caused streak defects and coating solution shortage that resulted in an uncoated portion in the form of a streak, independently of the level of the decompression degree, showing that the coating was unstable.

### Example 2

A coat of nickel plating of about 10 µm thick wherein Teflon fine particles are dispersed in a form of eutectoid was applied to a lip portion of an extrusion hopper coating apparatus, and a coating solution having the following composition was coated on a cellulose acetate web having a thickness of 125 µm and a width of 300 mm.

After coating under the conditions of coating speed of 100 m/min, decompression degree of -30 mmaq and coating density of 23 ml/m², no coating defects such as streak defects or the like were observed, resulting in stable coating.

The straightness in the web width direction of the plated lip portion of the extrusion hopper coating apparatus mentioned above was 2 µm and variation of the coating thickness after coating was about 5%.

| [Composition of coating solution] | parts by weight |
|---|---|
| Acetone | 70 |
| Isopropyl alcohol | 20 |
| Toluene | 10 |
| Cellulose acetate butylate | 0.5 |

### Comparative example 2

After coating with a coater of the extrusion hopper type which is of the same type as in Example 2 but is not subjected to the aforementioned plating on its lip portion, there were caused streak defects and coating solution shortage that resulted in an uncoated portion in the form of a streak, independently of the level of the decompression degree, showing that the coating was unstable.

### Comparative example 3

After the lip portion of the coater of an extrusion hopper type which is of the same type as in Example 2 was lined with Teflon-containing resins and ground instead of being subjected to the aforementioned plating, coating was conducted. As a result, no coating defects such as streak defects were caused but the straightness in the web width direction of the resin surface on the lip portion of the hopper was 12 µm and variation of coating thickness after coating was as high as about 30%.

### Example 3

A coat of nickel plating of about 10 µm thick wherein Teflon fine particles are dispersed in a form of eutectoid was applied to an inclined surface portion following the lip portion of an extrusion coating apparatus wherein each of upper and lower lip lengths is 2.5 mm, and a coating solution having the following composition was coated on a cellulose acetate web having a thickness of 125 µm and a width of 300 mm.

| [Composition of coating solution] | parts by weight |
|---|---|
| Acetone | 70 |
| Isopropyl alcohol | 20 |
| Toluene | 10 |
| Cellulose acetate butylate | 0.5 |

### (Coating conditions)

Coating speed: 60 m/min, decompression degree: -30 mmaq, coating density: 23 ml/m²

As a result, a length of a lower portion of a bead was almost equal to that of the lip positioned at an upstream side, and neither coating defects such as streak defects nor coating thickness problem were caused, resulting in stable coating.

Due to the invention, it has become possible to provide a coating method which may offer uniform coating that is free from streak defects, dropping defects, and coating defects such as comet defects, even when a coating solution having low surface tension and low viscosity is coated with a coating die of a slide hopper type or with a coating die of an extrusion type.

## Claims

1. A coating apparatus of a hopper type for coating one or more kinds of coating solutions on a running flexible support (2), said coating apparatus being provided with a slit (10) and a lip portion at the tip of a hopper,
characterized in that only an inclined surface following the lip portion is subjected to composite plating to be covered by a coat of the plating in which fluorine-containing resins are dispersed in a form of eutectoid such that the length of a bead upstream the slit (10)in the running direction of the flexible support (2) is adjusted to be nearly the same as that of the lip portion at the tip of the hopper at the upstream side of the slit (10) in the running direction of the support.

2. The coating apparatus according to claim 1, wherein a coat of plating wherein fluorine-containing resins are made in a form of eutectoid is based on non-electrolytic nickel plating utilizing chemical reaction.

3. The coating apparatus according to claim 1 or 2, wherein said fluorine-containing resin is Teflon.

4. The coating apparatus according to claim 1, 2 or 3, wherein a coat of plating is subjected, after being formed, to heat treatment at a temperature of not less than 200°C.

5. The coating apparatus according to claim 1, 2 or 3, wherein a coat of plating is subjected, after being formed, to heat treatment at a temperature of not less than 300°C.

6. The coating apparatus according to claim 1, 2 or 3, wherein a coat of plating is subjected, after being formed, to heat treatment at a temperature ranging from 300°C to 350°C.

7. A coating method comprising a step for coating one or more kinds of coating solutions on a running flexible support (2), wherein a coating apparatus is used which is provided with a slit (10) and a lip portion at the tip of a hopper and in which an inclined surface portion following the lip portion at the tip of a hopper is provided with a coat of composite plating wherein fluorine-containing resins are dispersed in a form of eutectoid,
characterized in that the coating is performed under the condition that a length of a portion of a bead (13) upstream the slit (10) in the running direction of the flexible support (2) is adjusted to be nearly the same as the length of the lip portion at the tip of the hopper at the upstream side of the slit (10) in the running direction of the flexible support (2) in that only the inclined surface following said lip portion is subjected to the composite plating.

8. The coating method according to claim 7, wherein the coat of plating is based on non-electrolytic nickel plating utilizing chemical reaction.

9. The coating method according to claim 7 or 8, wherein said fluorine-containing resin is Teflon.

10. The coating method according to claim 7, 8 or 9, wherein the coat of plating is subjected, after being formed, to heat treatment at a temperature of not less than 200°C.

## Patentansprüche

1. Beschichtungsvorrichtung eines Trichtertyps zum Beschichten eines (durch)laufenden Trägers (2) mit einer oder mehreren Arten von Beschichtungslösungen, welche Beschichtungsvorrichtung mit einem Schlitz (10) und einem Lippenteil an der Spitze eines Trichters versehen ist, dadurch gekennzeichnet, daß nur eine auf den Lippenteil folgende Schrägfläche einem Mehrstoff- oder Verbundplattieren unterworfen ist, so daß sie mit einem Überzug der Plattierung bedeckt ist, in welchem fluorhaltige Harze in Form eine Eutektoids dispergiert sind, derart, daß die Länge eines Wulstes stromauf des Schlitzes (10) in der Laufrichtung des flexiblen Trägers (2) so eingestellt ist, daß sie nahezu derjenigen des Lippenteils an der Spitze des Trichters an der Stromaufseite des Schlitzes (10) in der Laufrichtung des Trägers gleich ist.

2. Beschichtungsvorrichtung nach Anspruch 1, wobei ein Plattierüberzug, in welchem fluorhaltige Harze in die Form eines Eutektoids überführt sind, auf einem nichtelektrolytischen Nickelplattieren (Vernickeln) unter Nutzung einer chemischen Reaktion basiert.

3. Beschichtungsvorrichtung nach Anspruch 1 oder 2, wobei das fluorhaltige Harz Teflon ist.

4. Beschichtungsvorrichtung nach Anspruch 1, 2 oder 3, wobei ein Plattierüberzug nach seiner Erzeugung einer Wärmebehandlung bei einer Temperatur nicht unter 200°C unterworfen (worden) ist.

5. Beschichtungsvorrichtung nach Anspruch 1, 2 oder 3, wobei ein Plattierüberzug nach seiner Erzeugung einer Wärmebehandlung bei einer Temperatur nicht unter 300°C unterworfen (worden) ist.

6. Beschichtungsvorrichtung nach Anspruch 1, 2 oder 3, wobei ein Plattierüberzug nach seiner Erzeugung einer Wärmebehandlung bei einer Temperatur im Bereich von 300 - 350°C unterworfen (worden) ist.

7. Beschichtungsverfahren mit einem Schritt zum Beschichten eines (durch)laufenden flexiblen Trägers (2) mit einer oder mehreren Arten von Beschichtungslösungen unter Verwendung einer Beschichtungsvorrichtung, die mit einem Schlitz (10) und einem Lippenteil an der Spitze eines Trichters versehen ist und bei welcher ein auf den Lippenteil folgender Schrägflächenteil oder -bereich an der Spitze eines Trichters mit einem Überzug einer Mehrstoff- oder Verbundplattierung versehen ist, in welchem fluorhaltige Harze in Form eines Eutektoids dispergiert sind,
dadurch gekennzeichnet, daß das Beschichten unter der Bedingung durchgeführt wird, daß eine Länge eines Bereichs eines Wulstes (13) stromauf des Schlitzes (10) in der Laufrichtung des flexiblen Trägers (2) so eingestellt wird, daß sie nahezu der Länge des Lippenteils an der Spitze des Trichters an der Stromaufseite des Schlitzes (10) in der Laufrichtung des flexiblen Trägers (2) gleich ist, und daß nur die auf den Lippenteil folgende Schrägfläche der Verbundplattierung unterworfen ist.

8. Beschichtungsverfahren nach Anspruch 7, wobei der Plattierüberzug auf einem nichtelektrolytischen Nickelplattieren (Vernickeln) unter Nutzung einer chemischen Reaktion basiert.

9. Beschichtungsverfahren nach Anspruch 7 oder 8, wobei das fluorhaltige Harz Teflon ist.

10. Beschichtungsverfahren nach Anspruch 7, 8 oder 9, wobei der Plattierüberzug nach seiner Erzeugung einer Wärmebehandlung bei einer Temperatur nicht unter 200°C unterworfen wird bzw. worden ist.

## Revendications

1. Appareil d'application de type à trémie pour appliquer une ou plusieurs sortes de solutions d'application sur un support flexible mobile (2), ledit appareil d'application étant muni d'une fente (10) et une partie formant lèvre au bout d'une trémie,
caractérisé en ce que seule une surface inclinée suivant la partie formant lèvre est soumise à un placage composite destiné à être recouvert par une couche de placage dans laquelle des résines fluorées sont dispersées sous une forme d'eutectoïde de telle sorte que la longueur d'un bourrelet en amont de la fente (10) dans la direction d'avancement du support flexible (2) soit réglée de façon à être presque la même que celle de la partie formant lèvre au bout de la trémie au niveau du côté amont de la fente (10) dans la direction d'avancement du support.

2. Appareil d'application selon la revendication 1, dans lequel une couche de placage dans laquelle des résines fluorées sont sous une forme d'eutectoïde, est basée sur un placage de nickel non électrolytique utilisant une réaction chimique.

3. Appareil d'application selon la revendication 1 ou 2, dans lequel ladite résine fluorée est du téflon.

4. Appareil d'application selon la revendication 1, 2 ou 3, dans lequel une couche de placage est soumise, après avoir été formée, à un traitement à chaud à une température non inférieure à 200°C.

5. Appareil d'application selon la revendication 1, 2 ou 3, dans lequel une couche de placage est soumise, après avoir été formée, à un traitement à chaud à une température non inférieure à 300°C.

6. Appareil d'application selon la revendication 1, 2 ou 3, dans lequel une couche de placage est soumise, après avoir été formée, à un traitement à chaud à une température allant de 300 à 350°C.

7. Procédé d'application comprenant une étape pour appliquer une ou plusieurs sortes de solutions d'application sur un support flexible mobile (2), dans lequel un appareil d'application est utilisé qui est muni d'une fente (10) et d'une partie formant lèvre au bout d'une trémie et dans lequel une partie formant surface inclinée suivant la partie formant lèvre au bout d'une trémie est munie d'une couche de placage composite dans laquelle des résines fluorées sont dispersées sous une forme d'eutectoïde, caractérisé en ce que l'application est réalisée avec la condition qu'une longueur d'une partie d'un bourrelet (13) en amont de la fente (10) dans la direction d'avancement du support flexible (2) soit réglée de façon à être presque la même que la longueur de la partie formant lèvre au bout de la trémie au niveau du côté amont de la fente (10) dans la direction d'avancement du support flexible (2), en ce que seule la surface inclinée suivant ladite partie formant lèvre est soumise au placage composite.

8. Procédé d'application selon la revendication 7, dans lequel la couche de placage est basée sur un placage de nickel non électrolytique utilisant une réaction chimique.

9. Procédé d'application selon la revendication 7 ou 8, dans lequel ladite résine fluorée est du Téflon.

10. Procédé d'application selon la revendication 7, 8 ou 9, dans lequel la couche de placage est soumise, après avoir été formée, à un traitement à chaud à une température non inférieure à 200°C.
